

# UNITED STATES PATENT OFFICE.

LINDON WALLACE BATES, OF MOUNT LEBANON, NEW YORK.

## METHOD OF LOWERING THE VISCOSITY OF LIQUIDS.

1,382,456.

Specification of Letters Patent. Patented June 21, 1921.

No Drawing.

Application filed November 28, 1919. Serial No. 341,214.

To all whom it may concern:

Be it known that I, LINDON W. BATES, a citizen of the United States, and resident of Mount Lebanon, in the county of Columbia and State of New York, have invented a certain new and useful Improvement in Methods of Lowering the Viscosity of Liquids, of which the following is a specification.

10 This invention pertains to a liquid fuel and to the process for producing the same. More specifically it refers to a stable liquid fuel for burning purposes, produced by the combination of oil or tar, or liquid or mobile fuels comprising oil or tar, with dehydrated water gas tar or oil gas tar, which composite fuel possesses superior fuel qualities.

It is well known that many of the oils now used as fuel and tars suitable as combustibles are of such high viscosity at normal temperatures that they can be pumped relatively short distances only, unless heated, and that to be effectively "atomized" in existing burners they often have to be pre-heated above their flash point. The heavy oils from Mexico, Venezuela, Trinidad, and Sakhalin are especially subject to these disadvantages, which are usually even more accentuated when the oils have been

20 "topped", or the more volatile content partially or completely removed. For example, "Standard" oil from Mexico of specific gravity or rather density, 17.1° Baumé, has a flash point in a Pensky-Martens closed cup of 145° F., and a viscosity of 300.5° Engler at 70° F. Another like oil has a density of 15.4° Baumé, flash point 202° F., viscosity 715° Engler at 70° F. Certain Mexican residue has a density of 10° Baumé, flash

30 point of 374° F., and viscosity of 67° Engler at 200° F. A sample of Toltec oil has a specific gravity of 11.7° Baumé, flash point of 220° F. and viscosity of 166° Engler at 125° F., while another sample of this oil shows 12° Baumé, 124° F., and 375° Engler at 105° F., for density, flash point and viscosity respectively. "Richmond" California oil has a density of 17.1° Baumé, flash point of 228° F., and viscosity of 83.2° Engler at

40 70° F. ("Oil Burning", Lt. Com. J. J. Hyland, U. S. N., Proceedings of the American Society of Naval Engineers, 1914, vol. 26, p. 399 at p. 401). In order to reduce such heavy oils to the 8°-15° Engler required for spraying, that is to say "atomization", in the present atomizers of liquid fuel a heat

of as much as 230° F. and over is frequently required. Such heating often exceeds the flash point, which is exceedingly dangerous practice. ("Efficiency in the use of oil fuel", Wadsworth, U. S. Interior Department Pamphlet, 1918, p. 44).

The viscosity of liquid and mobile composite fuels having an oil base, is also high and resembles that of the viscous oils described above. Thus when a light oil is combined with a high percentage of powdered coal or other carbonaceous substance stabilized therein, the viscosity of the mixture closely approximates that of a heavy oil. On the other hand, the viscosity of a mixture of heavy oil with such powdered coal is not materially different from that of the heavy oil alone. Composite fuels of liquid hydrocarbon and pulverized carbonaceous substance duly treated for stability resemble in viscosity the heavy oils when the composite is in the liquid form and when extremely high percentages, such as over 50%, of solid carbons are used, the composites form pastes.

Endeavors have been made in the past to reduce the viscosity of heavy oils and to eliminate the consequential defects resulting therefrom. In Great Britain for example, it is the practice to blend with the Mexican oils, other oils of lesser viscosity. In the United States, heavy oil is generally used as it comes and the viscosity is reduced by heat. In a few recent instances in this latter country, where alone the Burton pressure stills are extensively used, pressure still oil or tar, so called, has been utilized as a "cut-back" or blending liquid. The term "pressure still oil or tar" refers to the residual left after cracking a paraffin base oil in pressure stills. There is not a large amount of this liquid available and its price is higher than that of heavy oil. It has recently been suggested that naphthalene may also be used as a cut-back, either alone or when dissolved with an oil itself derived from oil produced from gas house coal tar, blast furnace tar, coke-oven by-product coal tar, or from petroleum, oil residue, or schist oil. The proposed cut-back is then either naphthalene alone or naphthalene combined with a product of the distillation of coal or oil. It is also known in the art that middle fraction oils, such as creosote, and kerosene or hot wax tailings may be used. Kerosene, however, is at a disadvantage as a cut-back for

asphaltic base oils in that it tends to precipitate the asphaltic content. While technically suitable as cut-backs most of these liquids are economically unavailable. Thus 5 to use refinable light oils is a waste of natural resources. Partially refined oils are not available in large quantities for the purposes in view and when of low viscosity are usually dearer than heavy oils. For these 10 reasons, the reduction of the viscosity of heavy oils and of liquid or mobile composite fuels by the addition of liquids of low viscosity is not as attractive commercially as it may be made.

15 Chemical science, indeed, has now disclosed a cheap substance abundant in the United States and an easy way to reduce viscosity, and hence to lower the temperature at which asphaltic clots are formed and 20 the necessary preheat to enable the fuel to be atomized or sprayed. As a result of careful investigation, it has been found that water gas tar and oil gas tar, either of these alone or together, when properly dehydrated and combined with the liquid or mobile fuel whose viscosity is to be reduced, will serve the purpose. As such tars when produced carry sometimes up to 40% of water, and often up to 30%, it is essential to 25 dehydrate them so that the water content does not exceed about 10%. Dehydrated water and oil gas tars have a low viscosity. At 70° F. the viscosity of water gas tar is around 4.27° Engler. These two tars are 30 respectively produced from the "cracking" of oil vapors derived from treating coal and oil or oil alone with superheated steam. They are made in nearly all American gas plants, but not in all the British, where different systems of gas-producing are employed. To make water gas tar the "blue-gas" from coal treated with steam is combined with "gas oil." Oil gas tar is made from oil similarly "cracked." ("Asphalts 40 and Allied Substances," Abraham, 1918, p. 256 *et seq.*) They are broadly and precisely distinguished by chemists from the tars produced by the destructive distillation or partial combustion of coals or oils (same 45 p. 166, 262). Water gas tar and oil gas tar are chemically different from the oils and tars heretofore used as cut-backs, such as pressure still oil or tar, naphthalene, creosote, middle fraction oils generally and coal 50 tars produced in other ways. The ability of water or oil gas tar, when duly dehydrated, to reduce the viscosity of heavy oil or liquid composite fuels, to abolish the necessity of preheating many straight oils over their 55 flash point, to form with the oil or composite fuel a stable liquid, and finally to reduce a composite paste to a liquid have been qualities heretofore unappreciated in this relation and combinations not heretofore made. 60

65 The present invention consists, therefore,

in the product of the combination of oil or tar or composites containing such liquids, with dehydrated water or oil gas tar, or both, and in the process for suitably combining these components, and for regulating, 70 by the ratio of components and treatments, the viscosity, preheat necessary and stability. There are several distinct ways of producing the homogenous composite desired. The tar may be dehydrated before or during the 75 blending. A preferred way is to heat the components together to a temperature of from about 175° F. to 220° F. for a period of from one to three hours. The heating tank may be closed for safety if heating 80 above the flash point is required to blend the components and in the case of oils of low flash point less heat for a longer period may be employed. The treatment may also be given by passing the mixture through 85 any suitable stirring machine and heating the same during agitation. Agitation is preferably combined with heat treatments where expedition is required, but either agitation or heat alone if sufficiently extended 90 in duration and degree, will accomplish the result sought. The duration of the required treatment is necessarily variable, but must be such as will produce thorough commingling. In general, the greater the heat within reasonable limits and the more rapid the agitation, the less time is required to mix the liquids. The components may be mixed either in batches or by continuously pouring them together in proper proportions, using 95 careful calibration. The water or oil gas tar may be combined with composite fuels during the blending of the components of the latter fuel or prior thereto. The methods mentioned are by way of illustration and 100 not limitation.

It is instructive to give certain examples of the reduction of viscosity by the use of dehydrated tar of the varieties mentioned, using the heat blending treatment described 11 above. A typical topped Mexican oil has a viscosity of 600° Engler at 70° F. The introduction therewith of 20% by weight of dehydrated water gas tar reduces the viscosity of the mixture to 300° Engler, 40% 11 to 68° Engler, 60% to 29.5° Engler and 80% to 23° Engler. At 160° F. the viscosity of the same oil is 25.6° Engler and water gas tar is 1° Engler. The use of 20% of dehydrated water gas tar reduces the viscosity 12 of the composite at this temperature to 10.6° Engler which is sufficiently low to allow proper atomization. The introduction of 40% reduces the viscosity to 4.27° Engler, 60% to 3.1° Engler and 80% to 2° Engler. 12 These tars are superior as cut-backs to the other liquids available for this purpose. For example, at 160° F. 10% of pressure still oil only lowers the viscosity of Mexican reduced oil from 25.6° Engler to 18° Engler, 13

while the same amount of dehydrated water gas tar lowers it to 13° Engler.

The flash point of the same oil is 230° F., while that of the dehydrated water gas tar 5 is 158° F. and of the composite is 194° F. when 20% of dehydrated water gas tar is used. A composite consisting of 60% oil 10 40% tar has a flash point of 189° F. and of 40% oil 60% tar has a flash point of 185° F. 10 and 20% oil 80% tar has 158° F. It may be noted from these data that in the case of an 80% oil 20% tar composite, it is not necessary to preheat above the flash point to give adequate fluidity.

15 The stability of a mixture of oil or composite fuel with water or oil gas tar is adequate for all practical purposes. The two liquids form to some extent a true solution and to a considerable extent an emulsoid 20 and emulsion of notable natural stability. It must not be inferred, however, that all the ratios above stated can be used, and the fuel still retain adequate stability. Up to about 28% water gas tar, 32% oil and 40% 25 coal particles, by weight, may, for example, be stably combined for over a month.

Having thus stated the nature of my invention, what I claim is:

30 1. A stable liquid fuel comprising liquid hydrocarbon and dehydrated tar obtained

from the cracking of oil vapors derived from the treatment of coal and oil or oil alone with steam.

2. A stable liquid fuel consisting of particles of solid carbonaceous substance and 35 viscous mineral oil thinned with dehydrated water gas tar.

3. A stable liquid fuel consisting of liquid or mobile composite fuel, viscous liquid hydrocarbon and pulverized carbonaceous substance, thinned by dehydrated tar obtained 40 from the cracking of oil vapors derived from the treatment of coal and oil or oil alone with steam.

4. That method of producing a stable 45 liquid fuel which consists in adding dehydrated tar obtained from the cracking of oil vapors derived from the treatment of coal and oil or oil alone with steam to a liquid or mobile composite fuel, including 50 liquid hydrocarbon and pulverized carbonaceous substance, and in heating the components together for a considerable time at a temperature of from 175° F. to 220° F. until they adequately commingle. 55

Signed at New York city in the county of New York and State of New York this 3rd day of November, A. D. 1919.

LINDON WALLACE BATES.